

# UNITED STATES PATENT OFFICE.

CARLETON ELLIS, OF LARCHMONT, NEW YORK, ASSIGNOR, BY MESNE ASSIGNMENTS,  
TO CHADELOID CHEMICAL COMPANY, OF NEW YORK, N. Y., A CORPORATION OF  
WEST VIRGINIA.

## COMPOSITION FOR REMOVING WALL-PAPER.

1,084,201.

Specification of Letters Patent.

Patented Jan. 13, 1914.

No Drawing.

Application filed September 1, 1908. Serial No. 451,168.

To all whom it may concern:

Be it known that I, CARLETON ELLIS, a citizen of the United States, residing at Larchmont, in the county of Westchester and State 5 of New York, have invented certain new and useful Improvements in Compositions for Removing Wall-Paper, of which the following is a specification.

This invention relates to an improved 10 composition for the removal of old wall paper from the surfaces to which it is attached, and relates particularly to compositions capable of rapid penetration and effective softening of the adhesive so that a 15 plurality of coats or sheets of paper may be rapidly removed or stripped from the wall upon treatment with the said composition.

My invention has for its object the production or preparation of a composition 20 which has no appreciable action upon paint or varnish so that the composition may be employed without danger of injury to painted surfaces that might be moistened accidentally with the composition while using.

25 My invention comprises the use of three ingredients; viz:—water, a penetrating agent miscible with water and consisting preferably of alcoholic bodies, such as methyl acetone and the like, and a paste 30 softening agent such as an alkali or an acid, preferably the former.

It will be evident that a sufficient stage of dilution of the methyl acetone and the like and similar alcoholic bodies must be secured 35 in order to prevent action on paint and varnish which is an important consideration in the present invention, also in the case of the use of an alkaline soda or caustic alkali, it is preferable to use a quantity of saline 40 material such as sodium chlorid, sulfate of soda and the like in order to repress the action of the caustic as a paint and varnish removing agent so that the composition may be used with safety for removing wall paper 45 in proximity to painted and varnished surfaces.

The following illustrates the character of my improved composition:—One-half gallon of methyl acetone is diluted with water to make one gallon, and one-half ounce of commercial caustic soda is dissolved therein. To this mixture is added one pint of glycerin.

By varying the proportion of the pene-

trating agent different speeds of penetration 55 are secured. Too great a proportion of the penetrating agent weakens the action of the adhesive softening agent.

The addition of neutral salts such as common salt to the composition serves to further protect finish from accidental injury. A formula illustrative of the employment of 60 a finish-protecting ingredient comprises;—water, one gallon; methyl acetone, one quart; caustic soda, two ounces; and common salt, 65 a quantity sufficient to satyrate the mixture.

The process which I employ in the application of my improved composition consists in applying to the surface of the wall paper by means of a brush or spraying device a 70 sufficient amount of the removing composition to penetrate to the supporting wall; in allowing the composition to act for a short time until the adhesive is softened and then stripping the coating of wall paper from the 75 supporting surface. Subsequently, the surface of the supporting wall may be sponged with water if it is desired to remove any traces of the removing composition.

It will be evident that various modifications may be made in the manner of combining the ingredients above indicated and I do not limit myself to the exact proportions herein set forth, nor to the precise character 80 of the ingredients specified.

85 My invention comprises, as stated, a paste softening agent, an aqueous carrier for said agent, and a penetrating compound or material, so proportioned as to be safely used near painted surfaces. I have found that 90 ordinary aqueous solutions of various adhesive-softening agents greatly lack in penetrating properties. Water for instance may be applied to a heavy coating of wall paper, particularly the more expensive or highly 95 surfaced varieties of paper, for several hours time without penetrating to the adhesive. The addition of a penetrating agent, such as an alcoholic body, overcomes this difficulty and affords a commercially useful composition. Allied compounds, such as acetone and various other ketones, as well as various esters, such as ethyl acetate and the like also may be employed as penetrating agents.

100 For certain varieties of paste I prefer the composition acid and may acidify the composition by the use of mineral acids, such as sulfuric, hydrochloric, etc; or organic acids,

such as formic or acetic acids or methyl-  
and ethyl-sulfuric acid. While for certain  
other types of adhesives I prefer to use al-  
kali in very dilute solution, including the  
5 hydroxids and carbonates of soda, potash,  
and ammonia. I may also make use of such  
alkalis as barium hydrate or lime saccha-  
rate, but I prefer ordinarily to use caustic  
soda or potash.

10 What I claim is:

The composition for removing wallpaper  
consisting approximately of one quart of

methyl acetone, one gallon of water, two  
ounces of caustic soda and sufficient common  
salt to saturate the mixture and thereby sup-  
press the action of the caustic soda on paint  
and varnish.

In testimony whereof I have affixed my  
signature in presence of two witnesses.

CARLETON ELLIS.

Witnesses:

J. O. ROSER,  
JAS. D. REMSEN.